

## UNITED STATES PATENT OFFICE

LOUIS WEISBERG AND WILLARD F. GREENWALD, OF NEW YORK, N. Y., ASSIGNEES TO  
WEISBERG & GREENWALD, INC., OF NEW YORK, N. Y., A CORPORATION OF NEW  
YORK

## ELECTRODEPOSITION

No Drawing.

Application filed January 19, 1932. Serial No. 587,606.

This invention relates to electrodeposition, and particularly to the preparation of surfaces of lead or lead-containing alloys to receive electrodeposited coatings of metal.

5 Lead and lead alloys such as type metal and similar metals which are relatively soft are easily abraded, and consequently the exposed surfaces, when subjected to wear, are rapidly destroyed. This is particularly true in the case of stereotype plates and linotype slugs which are made by casting a molten alloy of lead containing small amounts of 10 hardening agents such as antimony. Printing surfaces of lead and lead alloys wear rapidly and are not adapted, therefore, for the 15 successful printing of large editions.

Attempts have been made heretofore to deposit wear-resisting metals electrolytically upon surfaces of lead and lead alloys, but 20 it is difficult to secure a proper bond between the electrodeposited metal and the underlying surface. Usually the coating metal cracks and chips from the surface and consequently the object of applying the coating 25 metal cannot be accomplished successfully.

It is the object of the present invention to provide a simple and effective procedure whereby wear-resisting metals can be deposited in a satisfactory manner upon the 30 surface of soft metals such as lead and alloys thereof to produce wear-resisting coatings which adhere to the underlying metal.

Another object of the invention is the provision of a method for depositing metals such 35 as copper, brass, nickel, or successive coatings of these metals upon printing plates and slugs and other similar objects of lead or lead-containing metals.

The object of the invention is accomplished 40 by suitably cleaning the surface of the article to be coated and then subjecting it as the anode for a short time to electrolysis in a neutral or alkaline solution. It is essential to the invention that the electrolyte employed 45 in the anodic treatment be slightly alkaline or neutral, since acid solutions tend to cause the formation of lead peroxide on a surface of lead or lead-containing alloy. After the brief anodic treatment, the surface can be 50 coated with copper, brass, or nickel or with

any of these metals successively by exposing it as the cathode in a suitable electrolyte under the usual conditions required for the deposition of the metals.

The invention will be described particularly with reference to the treatment of stereotype plates, although the procedure may be employed for the preparation for and deposition of metals electrolytically upon any article having an exposed surface of lead or a lead alloy. A stereotype plate may be prepared, for example, in the usual manner by casting a suitable type metal alloy having a basis of lead in the usual matrix. In the ordinary stereotype process a matrix of 55 paper is employed. The same principle is employed, however, in the preparation of linotype and monotype slugs and in the casting of ordinary type.

The stereotype plate, for example, is first 60 cleaned by immersing it in a hot electric cleaner solution, the plate being connected as the cathode with a voltage of approximately 6 volts. The composition of the electric 65 cleaner solution may vary. It should, however, be an alkaline solution strong enough 70 to remove grease and ink, if necessary. A solution containing 50 grams of trisodium phosphate per liter is satisfactory unless the plate is very dirty, in which case a stronger 75 solution may be employed. After the plate has been cleaned by exposure in the electric cleaner solution for a sufficient period, which will vary depending upon the amount of dirt 80 to be removed, it is brushed, if necessary, and 85 is then rinsed in running water.

The plate is then connected as the anode 90 in a suitable solution slightly alkaline or neutral. A satisfactory solution for this purpose contains approximately 50 grams per liter of sodium acetate. The plate is electrolyzed with a voltage of approximately 6 95 volts for a brief period, for example about 30 seconds, at ordinary room temperature. It is then removed from the bath and is ready for the plating operation.

Although we prefer to use a solution of sodium acetate as the electrolyte for the anodic treatment, it is possible to secure satisfactory results with various neutral and 100

alkaline solutions which do not form insoluble lead compounds. Solutions of the acetates, citrates and chlorides of the alkali metals are especially suitable for this treatment.

The plating procedure will vary depending upon the metal or metals to be deposited. For example, in plating with copper, we may employ the procedure suggested in "Principles 10 of Electroplating and Electroforming" by Blum and Hogaboom, second edition, page 228, employing a solution of copper (cuprous) cyanide about 22.5 grams per liter, sodium cyanide about 34.0 grams per liter, 15 and sodium carbonate about 15.0 grams per liter. The electrolysis may be conducted at a temperature of approximately 40° C. and a current density of about 14 amperes per square foot and for a time sufficient to deposit the desired amount of copper.

For brass plating, we may employ the procedure as set forth by Blum and Hogaboom at pages 379 to 389. Thus we may use a cyanide solution containing copper and zinc in 25 the ratio of 80:20 with a total metal content of at least 22.5 grams per liter and a free cyanide content about one-fourth the total of combined cyanide. To this bath may be added 30 to 60 grams per liter of sodium 30 carbonate. In this electrolyte at a temperature of about 40° C. the surface to be coated may be disposed as the cathode and subjected to the electric current with a cathode current density of about 2.8 amperes per square 35 foot. After a suitable interval which is best determined by consideration of the amount of brass to be deposited on the surface, the cathode is removed and is again thoroughly cleaned.

40 For nickel plating we may use a nickel solution as described by Blum and Hogaboom, page 260, solution 3, containing nickel sulphate about 200 grams per liter, nickel chloride about 45 grams per liter, and boric acid about 30 grams per liter, with a current 45 density of 14 to 47 amperes per square foot and at a temperature of 50° to 60° C. The plate obtained in this manner is hard and exceptionally adherent.

50 It will be understood that in carrying out the invention we may deposit any of the metals noted directly upon the surface of lead or lead-containing metal, or we may deposit a series of coatings, for example copper or brass, with nickel thereon.

55 Examination of the surface of the lead or lead-containing metal after exposure as the anode to the neutral or alkaline electrolyte shows that the surface is slightly etched. 60 The etching is not sufficient to affect the printing character of the surface, but it affords a bond for the overlying layer or layers of harder metal and prevents peeling and chipping of these layers. The invention is 65 especially advantageous in facilitating the

application of nickel to surfaces of lead containing metal.

Printing plates prepared and coated with nickel in the manner described will remain sharp and clear and will show little or no evidence of wear after producing many times the number of impressions which can be obtained ordinarily from type metal surfaces.

70 It is to be understood that the details of plating with the various metals form no part of the present invention and are subject to variation, the procedures described being merely typical of those well known in the art and adapted for the purpose of the invention, which depends more particularly upon the preparation of the surface to receive these metals and to permit the formation of a satisfactory bond between them and the underlying surface of lead or lead containing metal.

75 Various changes may be made in the details of the procedure without departing from the invention or sacrificing any of the advantages thereof.

80 We claim:

1. The method of preparing the surface of lead or a metal containing lead for coating by electrodeposition with another metal which comprises subjecting the surface as the anode to electrolysis in a neutral or alkaline electrolyte.

85 2. The method of preparing the surface of lead or a metal containing lead for coating by electrodeposition with another metal which comprises subjecting the surface as the cathode to an alkaline cleaning solution and 90 then as the anode to electrolysis in a neutral or alkaline electrolyte.

95 3. The method of preparing the surface of lead or a metal containing lead for coating by electrodeposition with another metal which comprises subjecting the surface as the anode to electrolysis in a neutral or alkaline electrolyte at a voltage of approximately 100 6 volts.

105 4. The method of preparing the surface of lead or a metal containing lead for coating by electrodeposition with another metal which comprises subjecting the surface as the anode to electrolysis in a solution of sodium acetate.

110 5. The method of preparing the surface of lead or a metal containing lead for coating by electrodeposition with another metal which comprises subjecting the surface as the anode to electrolysis in a solution containing 115 approximately 50 grams per liter of sodium acetate.

120 6. The method of improving the wear resistance of surfaces of lead and metal containing lead which comprises subjecting the surface as the anode to electrolysis in a neutral or alkaline electrolyte and thereafter electrodepositing on the prepared surface a harder coating metal.

125 7. The method of improving the wear re- 130

sistance of surfaces of lead and metal containing lead which comprises subjecting the surface as the cathode to an alkaline cleaning solution, then as the anode to electrolysis in a 5 neutral or alkaline electrolyte and thereafter electrodepositing on the prepared surface a harder coating metal.

8. The method of improving the wear re-  
sistance of surfaces of lead and metal con-

10

taining lead which comprises subjecting the surface as the anode to electrolysis in a neutral or alkaline electrolyte and thereafter electrodepositing on the prepared surface a plurality of layers of harder coating metals. 70

In testimony whereof we affix our signatures.

LOUIS WEISBERG.

WILLARD F. GREENWALD.

75

15

80

20

85

25

90

30

95

35

100

40

105

45

110

50

115

55

120

60

125